

W. O. STODDARD, JR.  
WATERPROOF FABRIC.  
APPLICATION FILED SEPT. 1, 1916.

Patented Oct. 9, 1917.

1,242,491.

Fig. 1.



Inventor  
William O. Stoddard Jr.  
By his Attorney  
Gifford & Bunn.

# UNITED STATES PATENT OFFICE.

WILLIAM O. STODDARD, JR., OF MADISON, NEW JERSEY, ASSIGNOR OF ONE-HALF TO  
FREDERIC E. KIP, OF MONTCLAIR, NEW JERSEY.

## WATERPROOF FABRIC.

1,242,491.

Specification of Letters Patent. Patented Oct. 9, 1917.

Application filed September 1, 1916. Serial No. 118,012.

*To all whom it may concern:*

Be it known that I, WILLIAM O. STODDARD, Jr., a citizen of the United States, residing at Madison, county of Morris, State of New Jersey, have invented certain new and useful Improvements in Waterproof Fabrics, of which the following is a specification.

My invention relates to a water-proof fabric which may be used for various purposes requiring such material as, for example, vehicle canopies, tops, curtains, clothing, etc.

Prior to my invention, so far as I am aware, one of the materials used for vehicle canopies or tops has consisted of two textile fabrics cemented together by a rubber cement. Such cement, however, deteriorates in a comparatively short time, ultimately disintegrates or crumbles and so loses its value both as a cement and as a water-proofing substance. Because of this characteristic of rubber cement the life of the material, when so made, is comparatively short. When such cement disintegrates the canopy or top leaks, and as the cement dries out the canopy material becomes hard and is broken by reason of the constant folding to which it is subjected. To remedy the defects incident to the use of rubber cement, particularly in its application to fabrics employed in the manufacture of vehicle tops, I have made an adhesive and water-proofing composition which composition is used in the manufacture of the material which forms the subject of the present application.

The adhesive and water-proofing composition used by me contains as its essential ingredients a nitro cellulose solution and a non-drying vegetable oil such as blown castor oil or blown rape-seed oil, preferably the former. Nitrated cotton is dissolved in any suitable solvent, preferably amyacetate, and the oil added to the solution and the mixture stirred by any suitable means, at normal temperature, until the mass is homogeneous. The proportions of nitrated cotton and oil may be varied to suit the particular fabric or use to which it is to be put. In practice I have used compositions containing one pound of nitrated cotton in solution to two and also three pounds of the preferred oil.

The cementing and water-proofing composition may be applied to the fabrics in various ways. In practice I have spread the composition on one fabric in quantity suffi-

cient for the purpose, and then laid the second fabric thereon, as the two pass between rolls of a calendering machine, sufficient pressure being applied to drive the composition into the texture of both fabrics, but not sufficient to drive it through them. In such method the two fabrics should be brought together before the composition has had time to set or become dry.

Another practice followed by me is to first spread upon both of the fabrics to be cemented together a composition containing substantially one part of cotton in solution to two parts of the preferred oil. The fabrics thus coated are air-dried for approximately two to three hours, or until the coatings have become "skin" dried. I then spread over one of the fabrics so coated a second composition containing substantially one pound of cotton in solution to three pounds of the preferred oil and lay thereon the other fabric, which has had an initial coat, sufficient pressure being applied to secure the desired result.

The blown vegetable oil used by me, and that which I prefer, is prepared by taking commercial raw castor oil having a specific gravity of about .9639 and, by the well-known method of blowing, reducing it so that its specific gravity will be in the neighborhood of 1.0294 to 1.0325, at a temperature of about 60° F. Blown rape seed oil, however, may be used.

In the accompanying drawings, in which Figure 1 is a side elevation and Fig. 2 is a diagrammatic view of the complete fabric, I have shown an apparatus which may be used for practising both of the methods above referred to. In this drawing the numeral 1 designates a suitable frame at one end of which is supported a roller 2 driven by any suitable means. At its other end, the frame supports a roller 3 driven by a belt 4 from the roller 2, or by means of gear and shaft from roller 2 to roller 3. Mounted above the roller 2 in blocks 5, slidably in standards 6, is a doctor blade 7. This blade may be adjusted angularly relatively to the roller 2 by a set screw 8. One of the component fabrics 9 of the finished product is run from a roll 10 over the roller 2 and as it passes under the doctor blade is coated with the described composition which collects in front of the blade in a mass, which mass is prevented from falling over the ends 110

of roller 2 by shields 11. From the roller 2, the fabric 9 passes between calender rolls 12 and 13, which rolls are supported in bearings mounted in guideways in standards 14. 5 The roll 12 may be adjusted vertically by gears 15, the lower of which is on a threaded shaft, as shown. The roll 12 may be heated in the usual manner. The bearings of roll 13 are supported upon springs 16. As the 10 fabric 9 enters the bight of the rolls 12 and 13 it meets the other component fabric 17 delivered from a roll 18. As the two fabrics pass between the rolls 12 and 13, they are subjected to the pressure to which the rolls 15 may be adjusted. The roll of fabric 10 is held under proper tension by a spring brake band, 19, and the roll 18 by a weight 20. From the calender rolls, the cemented product is carried over supports 21 around the 20 roller 3 and guide roll 22 to a take-up roll 23. To assist in drying the cement, if necessary or desired, the cemented fabric after passing between the calender rolls may be passed over a steam coil 24. 25 The method preferred by me is to give each of the fabrics 9 and 17 a preliminary coat of the cementing and water-proofing composition then, after being "skin" dried, to apply a final coat on one of the fabrics, 30 as 9. The solvent in the final coat is sufficient to unite or weld the two "skin" dried coats. The heat of the calender assists this union but the solvent in the final coat is the main agent to effect such result. In the 35 preferred method the final coat contains a greater percentage of oil than the first or "skin" dried coats so that when the nitro cellulose solution hardens, the non-drying oil in the final coat is sealed between two 40 layers of nitrated cotton. This feature of holding the oil permanently sealed from the air I regard as of importance in producing a commercial article, as the oil is thus protected from the disintegrating effects 45 of varying atmospheric conditions. The finished product is soft and pliable, im-

pervious to water and of such flexibility and durability as to render it suitable for use in the manufacture of water-proof articles such as canopies or tops and side curtains for automobiles and carriages. The product may, however, be used for any purpose for which it is adapted. 50

The fabrics to be united may be a drill and mohair as commonly used, or any other 55 suitable fabric. In Fig. 2 I have shown, diagrammatically, the two fabrics and the adhesive coats.

If desired the finished product may be subjected to the usual baking heat employed 60 in the manufacture of patent leather, this being from about 150° F. to 180° F. Such baking assists somewhat in hastening the drying of the nitro cellulose solution and the amalgamation of the composition with 65 the fabrics.

What I claim and desire to secure by Letters Patent of the United States is:—

1. An article of manufacture comprising two textile fabrics united by a non-drying 70 water-proof adhesive containing a blown vegetable oil.

2. An article of manufacture comprising two textile fabrics united by an adhesive containing nitro cellulose and a blown non- 75 drying oil.

3. An article of manufacture comprising two textile fabrics united by an adhesive containing nitro cellulose and a blown vegetable oil. 80

4. An article of manufacture comprising two textile fabrics united by an adhesive containing nitro cellulose and blown castor oil.

In testimony whereof I have hereunto 85 signed my name in the presence of two subscribing witnesses.

WILLIAM O. STODDARD, JR.

Witnesses:

D. A. DAVIES,  
CHARLES S. JONES.